

July 5, 1927.

1,634,923

L. H. THULLEN

TRANSFORMER

Filed July 15, 1924



## UNITED STATES PATENT OFFICE.

LOUIS H. THULLEN, OF UPPER MONTCLAIR, NEW JERSEY, ASSIGNOR, BY MESNE ASSIGNMENTS, TO J. C. THULLEN, OF LEETONIA, OHIO.

## TRANSFORMER.

Application filed July 15, 1924. Serial No. 726,067.

My invention relates to transformers and more particularly to transformers for use in radio reception apparatus, although the invention in its broader aspects is applicable to transformers for other purposes. In radio transformers one or more of the windings are commonly traversed by direct current from a battery or similar source of direct current. The alternating or oscillating voice or carrier current also traverses these windings. In order that the core does not become highly magnetized by the combination of the two currents, it is desirable by some means to increase the reluctance of the magnetic circuit. This reluctance should be a predetermined value dependent upon the amount of direct current traversing the windings so that the core is not magnetized beyond a given point which should be quite low in order that the same wave form of current is induced in the secondary as is in the primary.

In order that the shape of the current wave in the secondary be an exact duplicate, or nearly the shape, of the wave of the current in the primary, it is very desirable that the core of the transformer be very highly laminated. This, I have accomplished, by using very fine particles of iron (iron dust) mixed together with some form of a binder so that the iron particles are more or less separated magnetically by this binder. At the same time they are in sufficient close relation to each other to make a complete magnetic path. The amount of binder used depends upon the total reluctance that is desired in the magnetic circuit. For instance, should a calculation show that an air gap of a certain amount is desirable in the magnetic circuit then a sufficient percent of binder is used in connection with the iron dust to make the magnetic circuit equivalent to this air gap.

It is not new to use iron dust with a binder in other relationships but heretofore, so far as I am aware, this iron dust has been used with a minimum amount of binder so as to get an iron core with the minimum magnetic reluctance. However, I prefer to put in sufficient binder to increase the reluctance to a predetermined value for the reasons mentioned. At the same time this allows me to use a greater amount of binder thereby making the entire core structure more substantial. Heretofore the core of such an

article with a small amount of binder has been very fragile and quite expensive.

For certain purposes, therefore, I use a percentage of binder substantially greater than has heretofore been used, so far as I am aware, and the volume of the binder is preferably between about 2% and about 10% of the volume of the iron dust. Any suitable binder may be used such as silicate of soda.

Further and more specific objects, features and advantages will more fully appear from the detail description given below taken in connection with the accompanying sheet of drawings which form a part of this specification. In the drawings Fig. 1 is a plan view of a transformer embodying one form of my invention. Fig. 2 is a horizontal section taken on the line 2—2 of Fig. 3. Fig. 3 is a vertical section taken on the line 3—3 of Fig. 1. Fig. 4 is a view of the bottom of the transformer. Fig. 5 is a vertical section illustrating a modification and Fig. 6 is a similar section illustrating a further modification.

In the drawings 1 represents a suitable base of insulating material such as hard rubber or bakelite provided with downwardly extending supporting flanges 2. The base 1 is cut out on its top face as indicated in Figs. 3 and 4, and provided with four inwardly and downwardly extending lugs 3 separated by cut away spaces at 4. Supported on the lugs 3 is the bottom half 5 of a magnetic structure, which structure is in the form of a cup shaped member with a cylindrical upwardly extending wall 6, the bottom of the cup shaped member 5 having four slots 7 cut through it opposite the spaces 4 respectively. The cup shaped member 5 is provided with a centrally arranged cylindrical core 8 extending upwardly from the bottom of the cup. The cup shaped member 5 is moulded and made up of a mixture of iron dust (small iron particles) and any suitable binder such as silicate of soda as before mentioned. Over the member 5 is an inverted cup shaped member 9 provided with a downwardly extending cylindrical wall 10 having a rabbeted lower edge at 11 interlocking with a corresponding rabbeted edge on the wall 6. The member 9 is likewise molded and made up of a mixture of iron dust and a binder, and in order to strengthen and reinforce the members 5 and 9, I embed therein a series of wires 12, 13, 14 and 15,

the member 9 being also provided with a centrally arranged downwardly extending cylindrical core 16. The parts 8 and 16 form a central cylindrical core about which 5 are wound the primary turns or winding 17 and the secondary turns or winding 18 with insulating end members 19 and 20. The entire members 5 and 9 with the core parts 8 and 16 being molded of the mixture of iron 10 dust and binder, they form a magnetic structure which provides a closed magnetic circuit with a central core around which the turns are wound and which structure entirely surrounds and encloses the core and 15 the primary and secondary coils. This structure is, however, divided transversely into two or more removable parts for ease in assembling. The parts are held rigidly locked together by a bolt 21 passing vertically centrally through the magnetic core 20 and having a laterally turned end 22 at the bottom engaging under a transverse plate 23 the ends of which engage respectively under two of the lugs 3 on the base member 25 whereby upon tightening up on the nut 24 on the bolt the parts are pulled together and rigidly held in operative position. The base 1 is provided with binding posts 25 and 26 and leads 27 are connected to these binding 30 posts on the underneath side of the base and extend up through two of the slots 7 and in the member 5 to the secondary winding 18. The base 1 is also provided with two binding posts 28 and 29 and leads 30 are connected with these binding posts on the underneath side of the base and extend up through the other two slots 7 in the members 5 to the primary winding 17.

In Fig. 5 the upper inverted cup shaped member is shown as having a different form of core structure. Instead of an integral core structure of a mixture of iron dust and a binder, it is provided with a core structure formed of a cylindrical bundle of fine vertical iron wires 31. In Fig. 6 the structure is substantially the same except that the bundle of iron wires 32 forming the core structure, extend to the bottom of the lower cup shaped member 5, whereby 50 the entire core is made of iron wire.

The object of making the iron core partly of fine wire and partly of moulded iron dust is that I may be able to make a more substantial structure and still make a transformer with a small amount of eddy current losses. The fine iron wire will make a core better laminated than if made of sheet laminated steel. At the same time, the permeability of this part of the core will be quite high compared to its sectional area. This is desirable insomuch as it is desirable to get the primary and secondary windings as small as possible. The iron section exterior of that part of the iron circuit that 60 goes through the winding can have as large

a section as desirable as this part is exterior to the winding and in no way influences its size. The wires 12, 13, 14 and 15 may be either of nonferrous material or otherwise.

From the above it will be apparent that I have provided a transformer which is substantially iron clad in type. This is desirable since it shields the windings from stray fields from outside nearby apparatus.

While I have described my improvements in great detail and with respect to a preferred form thereof, many changes and modifications may be made and the invention embodied in widely different forms and 75 for various purposes without departing from the spirit and scope of the invention in its broader aspects. Hence I desire to cover all modifications and forms coming within the language or scope of any one or more of 80 the appended claims.

What I claim as new and desire to secure by Letters Patent, is:

1. A transformer having a substantially closed magnetic circuit comprising a central 90 core and a surrounding magnetic structure, and energizing turns about said core and surrounded by said surrounding magnetic structure, a substantial part of said magnetic circuit being made up of a mixture of 95 iron dust and a binder in which mixture the volume of the binder is from about 2% to about 10% of the volume of iron dust.

2. A transformer having a substantially closed magnetic circuit comprising a central 100 core and a surrounding magnetic structure, and energizing turns about said core and surrounded by said surrounding magnetic structure, said surrounding magnetic structure being made up of a mixture of iron 105 dust and a binder in which mixture the volume of the binder is from about 2% to about 10% of the volume of iron dust.

3. A transformer having a substantially closed magnetic circuit comprising a central 110 core and a surrounding magnetic structure, and energizing turns about said core and surrounded by said surrounding magnetic structure, said core being formed of a bundle of iron wires and a substantial part of 115 said magnetic circuit being made up of a mixture of iron dust and a binder in which mixture the volume of the binder is from about 2% to about 10% of the volume of iron dust.

4. A transformer having a substantial part of its magnetic circuit made up of a mixture of iron dust and a binder in which mixture the volume of the binder is from about 2% to about 10% of the volume of 125 iron dust, and said mixture having reinforcing members embedded therein.

5. A transformer having a substantially closed magnetic circuit comprising a central core and a surrounding magnetic structure,

70

75

80

85

90

95

100

105

110

115

120

125

130

- and energizing turns about said core and surrounded by said surrounding magnetic structure, said surrounding magnetic structure being made up of a mixture of iron dust and a binder in which mixture the volume of the binder is from about 2% to about 10% of the volume of iron dust, and said mixture having reinforcing members embedded therein.
10. A transformer having a substantially closed magnetic circuit comprising a central core and a surrounding magnetic structure, and energizing turns about said core and surrounded by said surrounding magnetic structure, the magnetic circuit structure being made in a plurality of parts for easy assembling and a substantial part thereof being made up of a mixture of iron dust and a binder.
15. A transformer having a substantially closed magnetic circuit comprising a central core and a surrounding magnetic structure, and energizing turns about said core and surrounded by said surrounding magnetic structure, the said surrounding structure being made in a plurality of separable parts for ease in assembling and a substantial part thereof being made up of a mixture of iron dust and a binder.
20. A transformer having a substantially closed magnetic circuit comprising a central core and a surrounding magnetic structure, and energizing turns about said core and surrounded by said surrounding magnetic structure, the said surrounding structure being made in a plurality of separable parts for ease in assembling and a substantial part thereof being made up of a mixture of iron dust and a binder.
25. A transformer having a substantially closed magnetic circuit comprising a central core and a surrounding magnetic structure, and energizing turns about said core and surrounded by said surrounding magnetic structure, the said surrounding structure being made in a plurality of separable parts for ease in assembling and a substantial part thereof being made up of a mixture of iron dust and a binder.
30. A transformer having a substantially closed magnetic circuit comprising a central core and a surrounding magnetic structure, and energizing turns about said core and surrounded by said surrounding magnetic structure, the said surrounding structure being made in a plurality of separable parts for ease in assembling and a substantial part thereof being made up of a mixture of iron dust and a binder, and said mixture having mechanical reinforcing means.
35. A transformer having a substantially closed magnetic circuit comprising a central core and a surrounding magnetic structure, and energizing turns about said core and surrounded by said surrounding magnetic structure, the said surrounding structure being made in a plurality of separable parts for ease in assembling and a substantial part thereof being made up of a mixture of iron dust and a binder, and means for locking said parts together.
40. A transformer having a substantially closed magnetic circuit comprising a central core and a surrounding magnetic structure, and energizing turns about said core and surrounded by said surrounding magnetic structure, the said surrounding structure being made in a plurality of separable parts for ease in assembling and a substantial part thereof being made up of a mixture of iron dust and a binder, and means for locking said parts together.
45. A transformer having a substantially closed magnetic circuit comprising a central core and a surrounding magnetic structure, and energizing turns about said core and surrounded by said surrounding magnetic structure, the said surrounding structure being made up of iron dust and a binder, and being divided transversely into a plurality of separable parts interlocking with one another.
50. A transformer having a substantially closed magnetic circuit comprising a central core and a surrounding magnetic structure, and energizing turns about said core and surrounded by said surrounding magnetic structure, the said surrounding structure being made up of iron dust and a binder, and being divided transversely into a plurality of separable parts interlocking with one another.
55. A transformer having a substantially closed magnetic circuit comprising a central core and a surrounding magnetic structure, and energizing turns about said core and surrounded by said surrounding magnetic structure, the said surrounding structure being made up of iron dust and a binder, and being divided transversely into a plurality of separable parts interlocking with one another.
60. A transformer having a substantially closed magnetic circuit comprising a central core and a surrounding magnetic structure, and energizing turns about said core and surrounded by said surrounding magnetic structure, the said surrounding structure having apertures in one end thereof through which leads extend to the windings of the transformer respectively.
65. A transformer having a substantially closed magnetic circuit comprising a central core and a surrounding magnetic structure, and energizing turns about said core and surrounded by said surrounding magnetic structure, a base of insulating material to
- surrounded by said surrounding magnetic structure, said surrounding structure being made up of iron dust and a binder, and being divided transversely into a plurality of separable parts interlocking with one another, and means passing axially through the transformer for holding said parts together. 70
12. A transformer having a substantially closed magnetic circuit comprising a central core and a surrounding magnetic structure, and energizing turns about said core and surrounded by said surrounding magnetic structure, said surrounding structure being made up of a mixture of iron dust and a binder, and being divided transversely into a plurality of separable parts interlocking with one another, and means passing axially through the transformer for holding said parts together, said mixture having mechanical reinforcing means and the volume of binder in the mixture being from about 2% to about 10% of the volume of iron dust therein. 75
13. A transformer comprising two cup shaped members facing one another and forming part of the magnetic circuit of the transformer and a magnetic core arranged centrally of said members. 80
14. A transformer comprising two cup shaped members facing one another and forming part of the magnetic circuit of the transformer and a magnetic core arranged centrally of said members, said cup shaped members being composed of a mixture of iron dust and a suitable binder. 85
15. A transformer having a core of magnetic material, a winding surrounding the same and an enclosing structure of magnetic material entirely surrounding said core and winding and forming part of the magnetic circuit of the transformer. 90
16. A transformer having a core of magnetic material, a winding surrounding the same and an enclosing structure of magnetic material entirely surrounding said core and winding and forming part of the magnetic circuit of the transformer, a substantial part of the magnetic circuit being formed of a mixture of iron dust and a binder. 100
17. A transformer having a substantially closed magnetic circuit comprising a central core and a surrounding magnetic structure, and energizing turns about said core and surrounded by said surrounding magnetic structure, said surrounding magnetic structure having apertures in one end thereof through which leads extend to the windings of the transformer respectively. 110
18. A transformer having a substantially closed magnetic circuit comprising a central core and a surrounding magnetic structure, and energizing turns about said core and surrounded by said surrounding magnetic structure, a base of insulating material to

which said structure is secured, primary and secondary binding posts on said base, and leads from said binding posts extending through the base of said surrounding structure to the primary and secondary of the transformer.

19. A transformer having a central core of magnetic material and an enclosing structure of magnetic material entirely surrounding said core, a base of insulating material and means passing through the core for securing the base to the core and magnetic structure, said core and magnetic structure forming the magnetic circuit of the transformer.

20. A transformer having a central core of magnetic material and an enclosing structure of magnetic material entirely surrounding said core, a base of insulating material and means passing through the core for securing the base to the core and magnetic structure, said core and magnetic structure forming the magnetic circuit of the transformer, and a substantial part of said magnetic circuit being made up of a mixture of iron dust and a binder in which mixture the volume of the binder is from about 2% to about 10% of the volume of iron dust.

21. A transformer having a central core of magnetic material and an enclosing structure of magnetic material entirely surrounding said core, a base of insulating material and means passing through the core for securing the base to the core and magnetic structure, said core and magnetic structure forming the magnetic circuit of the transformer, primary and secondary binding posts on said base, and leads therefrom extending through the bottom of the base and

said enclosing structure to the primary and secondary of the transformer.

22. A transformer having a substantially closed magnetic circuit comprising a central core and a surrounding magnetic structure, and energizing turns about said core and surrounded by said surrounding magnetic structure, a substantial part of said magnetic circuit being made up of a mixture of iron dust and a binder.

23. A transformer having a substantially closed magnetic circuit comprising a central core and a surrounding magnetic structure, and energizing turns about said core and surrounded by said surrounding magnetic structure, said core being formed of a bundle of iron wires and a substantial part of said magnetic circuit being made up of a mixture of iron dust and a binder.

24. A transformer having a substantially closed magnetic circuit comprising a central core and a surrounding magnetic structure, and energizing turns about said core and surrounded by said surrounding magnetic structure, said surrounding magnetic structure being made up of a mixture of iron dust and a binder.

25. A transformer having a substantially closed magnetic circuit comprising a central core and a surrounding magnetic structure, and energizing turns about said core and surrounded by said surrounding magnetic structure, said surrounding magnetic structure being made up of a mixture of iron dust and a binder and said mixture having reinforcing members embedded therein.

In testimony whereof I have signed my name to this specification.

LOUIS H. THULLEN.